

## UNITED STATES PATENT OFFICE.

HAROLD I. HUEY, OF SAYLESVILLE, RHODE ISLAND, ASSIGNOR TO SAYLES FINISHING PLANTS, INC., OF SAYLESVILLE, RHODE ISLAND, A CORPORATION OF RHODE ISLAND.

## PROCESS FOR PRODUCING TRANSPARENT EFFECTS UPON COTTON FABRICS.

No Drawing. Application filed May 19, 1922, Serial No. 562,243. Renewed September 30, 1924.

To all whom it may concern:

Be it known that I, HAROLD I. HUEY, a citizen of the United States, residing at Saylesville, in the county of Providence and

- 5 State of Rhode Island, have invented an Improvement in Processes for Producing Transparent Effects Upon Cotton Fabrics, of which the following description is a specification.
- 10 This invention relates to processes for producing transparent or "organdie" effects in cotton fabrics.

It is now well known that a cotton fabric treated with concentrated sulphuric acid 15 assumes a parchment-like effect, and that variations in the concentration of the sulphuric acid varies the effects produced. According to Mercer in 1844, this parchment-like character will be obtained if the sulphuric acid is of a concentration of from 20 49.5° to 53.5° Bé. The action of the sulphuric acid is also known to be more intense when the cotton fabric has been previously mercerized and the acid concentration 25 is over 50½° Bé. It is also known that transparent effects may be produced in cotton goods by subjecting the fabric to the repeated action of sulphuric acid of over 30 50½° Bé. and concentrated alkali lye, and that regulation of temperature in some cases to a point about 0° C. or less may still further modify the effect produced.

To secure the desired result in any case 35 requires nicety of control of the sulphuric acid concentration, since variation in this causes variations in the character and appearance of the product. One of the purposes of the present invention therefore is to provide a process for the production of 40 transparent effects in woven cotton fabrics in which a wide range of variation in the concentration of the acid employed may be possible without material variation in the resulting product.

45 Where the concentration of the sulphuric acid must be maintained constant and at a substantially fixed point, or between very narrow limits, the watchful care of skilled operatives is required to avoid damage or 50 variations in the woven fabric under treatment. One of the important features of the present invention consists in a process for producing transparent effects in woven cot-

ton fabrics which will not cause damage or material variations in the final product even 55 though variations of wide range occur in the concentration of the acid employed.

It has heretofore been known that wool-like effects may be produced in cotton fabrics by treatment with hydrochloric acid or phosphoric, or even with nitric acid, but similar restricted limitations in the range of variations of concentration exist as in the case with sulphuric acid. I have found that sulphuric acid and hydrochloric acid united 60 in determined proportions produces a hydrochloric-sulphuric acid having an effect on woven cotton fabrics different from either, and that where a cotton fabric is treated by hydrochloric-sulphuric acid a fine, uniform, 65 transparent organdie results, and that a wide range in variation of concentration of the acid may occur without material variation in the uniform texture of the resulting product. This permissible wide range of 70 concentration of the hydrochloric-sulphuric acid is of great importance in furnishing a wider range of control, elimination to a degree at least of the watchful attention of 75 skilled experts, and lending commercial 80 practicability to the process.

In practicing the process in accordance with the present invention, the woven cotton fabric may be boiled, bleached and dried and then mercerized and again dried, or it 85 may be mercerized, then boiled, bleached and dried. In any event, however, it is desirable to remove from the woven cotton fabric the natural gums and waxes inherent in the fibre and also to remove the sizing placed 90 upon the fabric during the finishing operation following weaving.

The process may be practiced on either mercerized or unmercerized woven cotton fabric but preferably the woven cotton fabric will be mercerized, because such preliminary mercerization causes the yarn to become more even and of a uniform texture, while the fabric as a whole is rendered more susceptible to the acid treatment to follow. 95

In forming the acid combination, the hydrochloric acid or phosphoric acid, each of which has a well-known parchmentizing effect, but of a character different from that of sulphuric acid, and whichever be used, 100 preferably hydrochloric acid, the com-

mercial quality of such acid will be combined with sulphuric in determined proportions to form an hydrochloric-sulphuric acid. The proportion of the acids well suited for 5 the purpose is sulphuric acid of about 56° Bé. concentration, for instance, combined with the commercial hydrochloric acid in the proportion of one part of each, the result being with respect to such proportions 10 that the hydrochloric-sulphuric acid will be of a concentration of about 41° Bé. Higher concentration of the mixture, for instance, as high as 50° Bé., may be reached by mixing the sulphuric acid and hydrochloric acid 15 together in a proportion of about 3½ parts of sulphuric acid to one part of hydrochloric acid.

The acid mixture thus obtained may vary 20 in concentration between wide ranges, as for instance, with respect to the above mixture from 41° Bé. to 50° Bé., and yet produce a clear, uniform, "organdie" effect on cotton fabric treated by it.

The woven cotton fabric whether previously mercerized or not, is then subjected 25 to the hydrochloric-sulphuric acid, preferably of a concentration of from 41° to 50° Bé. and is then preferably remercerized to increase the finished appearance and "organdie" effect of the final produce.

30 The fabric is then washed and dried and presents a transparent, uniform texture.

What is claimed is:

The described process for producing transparent effects on woven cotton fabric, consisting in subjecting the woven fabric to the action of hydrochloric-sulphuric acid of a concentration of from 41° to 50° Bé. formed by a combination of from one to three and one-third parts sulphuric acid, one part of hydrochloric acid, and then washing and 35 drying the treated fabric.

In testimony whereof, I have signed my name to this specification.

HAROLD I. HUEY.